



US005879408A

# United States Patent [19]

Kubo et al.

[11] Patent Number: **5,879,408**[45] Date of Patent: **Mar. 9, 1999**

[54] **METHOD OF STAINPROOFING  
CELLULOSE FIBERS AND STAINPROOFED  
PRODUCT**

[75] Inventors: **Motonobu Kubo; Takashi Enomoto**,  
both of Osaka, Japan

[73] Assignee: **Daikin Industries Ltd.**, Osaka, Japan

[21] Appl. No.: **849,842**

[22] PCT Filed: **Dec. 14, 1995**

[86] PCT No.: **PCT/JP95/02559**

§ 371 Date: **Jun. 12, 1997**

§ 102(e) Date: **Jun. 12, 1997**

[87] PCT Pub. No.: **WO96/18764**

PCT Pub. Date: **Jun. 20, 1996**

[30] **Foreign Application Priority Data**

Dec. 15, 1994 [JP] Japan ..... 6-311635

[51] **Int. Cl.<sup>6</sup>** ..... **D06M 13/188**; D06M 15/277

[52] **U.S. Cl.** ..... **8/120**; 8/121; 8/116.1;  
427/389.9; 427/391; 427/392; 427/394;  
427/393.4; 427/395; 427/396; 442/94; 442/95;  
428/364; 428/365

[58] **Field of Search** ..... 8/120, 121, 116.1;  
427/389.9, 391, 392, 394, 395, 396, 393.4;  
442/94, 95; 428/364, 365

[56] **References Cited**

U.S. PATENT DOCUMENTS

1,861,320 5/1932 Rheiner ..... 8/121  
3,574,791 4/1971 Sherman et al. .

3,919,183 11/1975 Jager et al. ..... 526/245

FOREIGN PATENT DOCUMENTS

02277887 11/1990 Japan .

04068006 3/1992 Japan .

06116340 4/1994 Japan .

5235033 9/1997 Japan .

OTHER PUBLICATIONS

A.J. Hall, "The Standard Handbook of Textiles," pp. 43-53, (month unknown), 1975.

A.J. Hall, "The Standard Handbook of Textiles," pp. 49-50, (month unknown), 1975.

Primary Examiner—Alan Diamond  
Attorney, Agent, or Firm—Birch, Stewart, Kolasch & Birch,  
LLP

[57] **ABSTRACT**

Stainproofing properties are imparted to a cellulose fiber by 1) esterifying a part of hydroxyl groups of the cellulose fiber in a heterogeneous reaction system and 2) subjecting the partially esterified cellulose fiber to a stainproofing treatment with an aqueous solution or emulsion of a copolymer having repeating units derived from a fluoroalkyl group-containing polymerizable compound and a compound represented by the general formula:



wherein X is  $-\text{CH}(\text{CH}_3)-\text{CH}_2-$  or  $-\text{CH}_2-\text{CH}(\text{CH}_3)-$ ;  
Y is  $-\text{CH}_2\text{CH}_2-$ ;  $\text{R}^1$  is a hydrogen atom or a methyl group;  
 $\text{R}^2$  is a hydrogen atom or an alkyl group having 1 to 8 carbon atoms; and each of m and n is an integer of 0 to 50, provided that the total of m and n is an integer of 1 to 70.

**14 Claims, No Drawings**



## 3

-continued

$\text{CF}_3(\text{CF}_2)_7(\text{CH}_2)_4\text{OCOCH}=\text{CH}_2,$   
 $\text{CF}_3(\text{CF}_2)_7\text{SO}_2\text{N}(\text{CH}_3)(\text{CH}_2)_2\text{OCOC}(\text{CH}_3)=\text{CH}_2,$   
 $\text{CF}_3(\text{CF}_2)_7\text{SO}_2\text{N}(\text{C}_2\text{H}_4)(\text{CH}_2)_2\text{OCOCH}=\text{CH}_2,$   
 $\text{CF}_3(\text{CF}_2)_7\text{CONH}(\text{CH}_2)_2\text{OCOCH}=\text{CH}_2,$   
 $(\text{CF}_3)_2\text{CF}(\text{CF}_2)_4(\text{CH}_2)_3\text{OCOCH}=\text{CH}_2,$   
 $(\text{CF}_3)_2\text{CF}(\text{CF}_2)_4\text{CH}_2\text{CH}(\text{OCOCH}_3)\text{CH}_2\text{OCOC}(\text{CH}_3)=\text{CH}_2,$   
 $(\text{CF}_3)_2\text{CF}(\text{CF}_2)_4\text{CH}_2\text{CH}(\text{OH})\text{CH}_2\text{OCOCH}=\text{CH}_2,$   
 $\text{CF}_3(\text{CF}_2)_9(\text{CH}_2)_2\text{OCOCH}=\text{CH}_2,$

## 4

$\text{CH}_2=\text{C}(\text{CH}_3)\text{COO}(\text{CH}_2\text{CH}_2\text{O})_9\text{CH}_3\text{CH}_2=\text{C}(\text{CH}_3)$   
 $\text{COO}(\text{CH}_2\text{CH}(\text{CH}_3)\text{O})_{12}\text{H}/3\text{-chloro-2-hydroxypropyl}$   
 $\text{methacrylate/glycerol monomethacrylate,}$

5 a combination described in Example 1 of Japanese Patent Kokoku Publication No. 35033/1977:

$\text{CH}_2=\text{C}(\text{CH}_3)\text{COO}(\text{CH}_2\text{CH}_2\text{O})_9\text{H}/\text{CH}_2=\text{C}(\text{CH}_3)\text{COO}$   
 $(\text{CH}_2\text{CH}_2\text{O})_{4.5}\text{H}/\text{methacrylonitrile}/\text{CH}_2=\text{C}(\text{CH}_3)$   
 $\text{COOCH}_2\text{CH}_2\text{OH};$

10 a combination described in Example 1 of Japanese Patent Kokai Publication No. 68006/1992:



-continued

$\text{CF}_3(\text{CF}_2)_9(\text{CH}_2)_2\text{OCOC}(\text{CH}_3)=\text{CH}_2,$   
 $\text{CF}_3(\text{CF}_2)_4\text{CONH}(\text{CH}_2)_2\text{OCOC}(\text{CH}_3)=\text{CH}_2,$   
 $\text{CF}_2\text{Cl}$   
 $\text{CF}_3$   
 $\text{CF}(\text{CF}_2)_4\text{CONH}(\text{CH}_2)_2\text{OCOCH}=\text{CH}_2,$   
 $\text{H}(\text{CF}_2)_{10}\text{CH}_2\text{OCOCH}=\text{CH}_2,$  and  
 $\text{CF}_2\text{Cl}(\text{CF}_2)_{10}\text{CH}_2\text{OCOC}(\text{CH}_3)=\text{CH}_2$

As the compound represented by the above general formula (I) as the other component of the copolymer used in the present invention, a compound wherein each of n and m is 1 to 25 is preferred. These compounds may be used alone or in combination thereof.

The copolymer used in the present invention contains the fluoroalkyl group-containing polymerizable compound in an amount within the range usually from 5 to 95% by weight, preferably from 30 to 80% by weight, more preferably from 40 to 70% by weight, based on the total weight of the copolymer. When the amount of the fluoroalkyl group-containing polymerizable compound exceeds 95% by weight, the soil release property is insufficient. On the other hand, when the amount is smaller than 5% by weight, the oil repellency is insufficient.

An average molecular weight of the copolymer is normally from 1,000 to 1,000,000 (measured by a gel permeation chromatography (GPC)).

When the durability is particularly required, the copolymer may be copolymerized by adding a crosslinking monomer such as 3-chloro-2-hydroxypropyl (meth)acrylate, N-methylol (meth)acrylamide, diacetone (meth)acrylamide, glycidyl (meth)acrylate, glycerol mono(meth)acrylate, (meth)acrylic acid, isocyanate group-containing (meth)acrylate, blocked isocyanate-containing (meth)acrylate and the like. It is also possible to copolymerize (meth)acrylonitrile, vinyl chloride, vinylidene chloride,  $\text{C}_1\text{--C}_{18}$  alkyl ester of acrylic acid or (meth)acrylic acid, styrene, benzyl (meth)acrylate, vinyl alkyl ketone, vinyl alkyl ether, isoprene, butadiene, chloroprene and the like.

These third monomers are used in an amount within the range usually from 0 to 40% by weight, preferably from 0 to 25% by weight, more preferably from 0 to 15% by weight, based on the total weight of the copolymer.

Examples of the preferred combination of the monomers include a combination described in Example 1 of Japanese Patent Kokai Publication No. 116340/1994:

25 In order to further improve the water repellency and the oil repellency, a water- and oil-repellent (e.g. TG-521 (manufactured by Daikin Industries Ltd.)) can be mixed with the copolymer of the present invention in any proportion. In case of using the water- and oil-repellent, a weight ratio of the copolymer to the water- and oil-repellent active component is preferably from 10:0 to 10:50.

30 In order to obtain the copolymer of the present invention, various methods and conditions of the polymerization reaction can be optionally selected, and any of various polymerization methods such as a bulk polymerization, a solution polymerization, a suspension polymerization, an emulsion polymerization, and a radiation polymerization can be used. 35 For example, there can be used a method which comprises emulsifying a mixture of copolymerizable compounds in water in the presence of a surfactant, and copolymerizing the mixture with stirring. As a polymerization initiator for the reaction system, various initiators such as a peroxide initiator, an azo initiator and a persulfuric acid initiator can be used. Since a polyalkylene glycol acrylate or methacrylate acts as a surfactant, it is not necessary to use the surfactant but various emulsifiers such as an anionic emulsifier, a cationic emulsifier and a nonionic emulsifier 45 may be optionally used.

40 It is possible to perform a solution polymerization by an action of the polymerization initiator (e.g. a peroxide or azo compound which is soluble in the used organic solvent, or an ionizing radiation) after dissolving monomers in a suitable 50 organic solvent. Examples of the solvent which is suitable for the solution polymerization include acetone, methyl ethyl ketone, isopropanol, ethylcellosolve, propylene glycol monomethyl ether, dipropylene glycol monomethyl ether, diglyme, triglyme and the like.

55 A stainproofing agent having any form such as an emulsion, a solvent solution, and an aerosol can be prepared from the obtained copolymer according to a conventional method.

60 A method of applying the stainproofing agent containing the copolymer as an active component may be appropriately selected according to the type of a treated material, the purpose of use and the form of the stainproofing agent. In case of the aqueous emulsion or solvent solution, it may be applied to the surface of a material to be treated by a known method such as a spray, a dipping and a coating, followed by 65 drying. If necessary, a curing may be conducted. In case of the aerosol, it may only be sprayed to the material to be

treated, followed by drying. Furthermore, antistatic agents, flame retardants, creaseproofing agents and other polymers may optionally be added to the copolymer of the present invention.

An amount of the copolymer to be applied to the cellulose fiber wherein a part of hydroxyl groups is esterified by the method of the present invention is usually from 0.1 to 10 parts by weight, based on 100 parts by weight of the treated material (cellulose fiber).

#### PREFERRED EMBODIMENT OF THE INVENTION

The present invention will be illustrated by Examples and Comparative Examples which do not limit the present invention. In the Examples and Comparative Examples, "%" is % by weight, unless otherwise stated.

##### (1) Water repellency and oil repellency

The water repellency and oil repellency shown in the following Examples and Comparative Examples were determined by the following test methods.

The water repellency is expressed by the water repellency No. (see Table 1) determined by the spray method according to JIS (Japanese Industrial Standard) L-1092. The oil repellency is determined by dropping 0.05  $\mu$ L of a test solution shown in Table 2 on the surface of a test cloth and observing the penetration state of the drops after 30 seconds (AATCC-TM118-1983).

TABLE 1

| Water repellency No. | State                                       |
|----------------------|---------------------------------------------|
| 100                  | No wet on the surface                       |
| 90                   | Slight wet on the surface                   |
| 80                   | Partial wet on the surface                  |
| 70                   | Wet on the surface                          |
| 50                   | Wet over the whole surface                  |
| 0                    | Complete wet on the front and back surfaces |

TABLE 2

| Oil repellency | Test solution                        | Surface tension (dyne/cm, 25° C.) |
|----------------|--------------------------------------|-----------------------------------|
| 8              | n-Heptane                            | 20.0                              |
| 7              | n-Octane                             | 21.8                              |
| 6              | n-Decane                             | 23.5                              |
| 5              | n-Dodecane                           | 25.0                              |
| 4              | n-Tetradecane                        | 26.7                              |
| 3              | n-Hexadecane                         | 27.3                              |
| 2              | n-Hexadecane/Nujol (35/65 by weight) | 29.6                              |
| 1              | Nujol                                | 31.2                              |
| 0              | Inferior to 1                        | —                                 |

##### (2) Soil release property (SR property)

The soil release property (SR property) is conducted as follows. A test cloth is spread on a filter paper laid horizontally and 0.1  $\mu$ L of a dirty motor oil is dropped. After covering a polyethylene sheet thereon, a weight of 2 kg is put on the polyethylene sheet. After 60 seconds, the weight and the polyethylene sheet are removed. After standing at room temperature for 1 hour, the test cloth is washed with using 60 g of a detergent (Super Zabu: trade name) under the conditions of a bath volume of 35 liter and a liquid temperature of 40° C. for 10 minutes in an electric washing machine, rinsed and then air-dried. The state of the dried test cloth is expressed by a corresponding evaluation class shown in Table 3.

TABLE 3

| Evaluation class | Evaluation criteria        |
|------------------|----------------------------|
| 1.0              | Remarkable stain remains   |
| 2.0              | Considerable stain remains |
| 3.0              | Slight stain remains       |
| 4.0              | Unnoticeable stain remains |
| 5.0              | No stain remains           |

Examples of esterifying a part of hydroxyl groups of the cellulose fiber will be shown below.

##### Preparative Example 1 (acetylation in liquid phase)

Three cotton cloths (50 cm×50 cm) were put in a wide-mouthed bottle, and then 3 liter of a mixed solution of acetic anhydride/pyridine (20/80 vol./vol.) was poured into the bottle to entirely immerse the cotton cloths. After capping the bottle loosely with a glass stopper, the bottle was allowed to stand in a hot water at 60° C. for 8 hours.

After the completion of the reaction, the treated cloths were washed with water until the wash liquid does not exhibit acidity. Further the cloths were boiled for 30 minutes for stabilization. A content of bound acetic acid was measured according to a Frank Howlett's method [Journal of Textile Institute (J. Text. Inst.), 35 T1(1944)]. As a result, it was 9.2%. That is, the degree of substitution (DS) was 0.266.

The degree of substitution (DS) after acetylation was determined in the following manner.

When A is a content of bound acetic acid (%), the following equation is established.

$$A = (60 \times DS \times 100) / (162 + 42DS)$$

This equation is modified to give the following equation.

$$\text{Degree of substitution (DS)} = (3.86 \times A) / (142.9 - A)$$

##### Preparative Example 2 (acetylation in vapor phase)

A cotton cloth (30 cm×30 cm) was immersed in 0.1N sulfuric acid at room temperature for 10 minutes, squeezed to a third to evaporate water until the water content was 50%, and then brought into contact with vapor of acetic anhydride in a desiccator at 20° C. for 10 hours. After the completion of the reaction, the degree of substitution was determined after treating according to the same manner as in Preparative Example 1. As a result, it was 0.247.

##### Preparative Example 3 (acetylation in vapor phase)

According to the same manner as in Preparative Example 2 except that an aqueous zinc sulfate solution (0.1 mol/L) was used in place of sulfuric acid and the time and the temperature for contacting with acetic anhydride vapor were changed to 3.5 hours and 60° C., respectively, the operation was conducted to obtain the acetylated cotton having degree of substitution of 0.78.

##### Preparative Example 4 (propionylation in liquid phase)

Ten cotton cloths (30 cm×30 cm) (100 g in total) were dried until the water content became 5%. The cotton cloths were immersed in 1.5 liter of propionic acid at room temperature for 10 hours. Then, these cotton cloths were squeezed until the total weight became 250 g. These pre-treated cotton cloths were put at 40° C. in a mixture prepared

by previously mixing 400 g of propionic acid, 50 g of zinc chloride and 400 g of propionic anhydride. The cotton cloths were removed after 20 minutes, put in a large amount of water, washed with water repeatedly and air-dried.

An amount of bonded propionic acid was determined in the following manner.

About 1 g of an air-dried esterified sample was dried over phosphorus pentaoxide in a vacuum desiccator, precisely weighed and charged in a 200 mL glass-stoppered Erlenmeyer flask. After adding 50 mL of a 0.5N methanolic potassium hydroxide solution, the mixture was saponified by allowing to stand at room temperature for 48 hours. Then, the amount of bonded propionic acid was determined after back titration with 0.5N hydrochloric acid.

The degree of substitution of the resulting propionylated cotton was 0.18.

#### Preparative Example 5 (palmitylation)

Twenty cotton cloths (about 160 g) (20 cm×30 cm) dried over phosphorus pentaoxide under a reduced pressure to give a constant weight were weighed. 320 g of pyridine and 2,500 mL of acetone were added to the cloths. Then, a solution of palmitoyl chloride ( $C_{15}H_{31}COCl$ , 980 g) in acetone (1600 mL) was added over 20 minutes and the mixture was reacted under reflux in a glass reaction vessel equipped with a reflux condenser for 90 minutes.

After cooling, the cotton cloths were washed three times with methanol and with acetone, alternately, and were extracted with acetone for 24 hours by a Soxhlet extractor. Acetone was removed to give a constant weight under a reduced pressure, and the cloths were precisely weighed. The degree of substitution determined by considering an increase in weight before and after the reaction to be caused by a palmitoyl esterification was 0.046.

Hereinafter, Preparative Examples of the stainproofing agent used in the second step will be shown.

#### Preparative Example 6

A compound (20 g) represented by  $CF_3CF_2(CF_2CF_2)_nCH_2CH_2OCOC(CH_3)=CH_2$  (a mixture of compounds wherein

n is 3, 4 and 5 in a weight ratio of 5:3:1),

10 g of  $CH_2=C(CH_3)COO(CH_2CH_2O)_9CH_3$ ,

5 g of  $CH_2=C(CH_3)COO(CH_2CH(CH_3)O)_{12}H$ ,

4 g of  $CH_2=C(CH_3)COOCH_2CH(OH)CH_2Cl$ ,

1 g of  $CH_2=C(CH_3)COOCH_2CH(OH)CH_2OH$  and 60 g of isopropanol were charged in a four-necked flask equipped

with a mercury thermometer and a stirrer of a tetrafluoroethylene crescent-shaped stirrer, and then sufficiently emulsified by stirring under a nitrogen flow. After the atmosphere in the flask was sufficiently replaced by blowing nitrogen for about 1 hour, 0.1 g of azobisisobutyronitrile was charged

and the copolymerization reaction was conducted at 70°C. with stirring for 10 hours. A gas chromatography analysis revealed that a conversion rate of the copolymerization reaction is not smaller than 97%. This conversion rate showed that the proportion of each repeating unit in the resulting copolymer is almost the same as that of the charged monomers. After the completion of the reaction, 40 g of isopropanol and 60 g of deionized water were charged to dilute the reaction liquid. The resulting copolymer liquid contained 19.5% by weight of a copolymer. A molecular weight of the copolymer was 12,000 (in terms of styrene) according to a gel permeation chromatography (GPC).

#### Preparative Example 7

A compound (70 g) represented by  $CF_3CF_2(CF_2CF_2)_nCH_2CH_2OCOCH=CH_2$  (a mixture of compounds wherein n is 3, 4 and 5 in a weight ratio of 5:3:1),

#### 8

25 g of  $CH_2=C(CH_3)COO(CH_2CH_2O)_9CH_3$ ,

5 g of

and



400 g of isopropanol were charged in a 1 liter four-necked flask equipped with a mercury thermometer and a stirrer of a tetrafluoroethylene crescent-shaped stirrer, and then sufficiently dispersed by stirring under a nitrogen flow. After the atmosphere in the flask was sufficiently replaced by blowing nitrogen for about 1 hour, 1.0 g of azobisisobutyronitrile was added and the copolymerization reaction was conducted under a nitrogen flow at 70°C. for 10 hours. A gas chromatography analysis revealed that a conversion rate of the copolymerization reaction is not smaller than 99%. This conversion rate showed that the proportion of each repeating unit in the resulting copolymer is almost the same as that of the charged monomers. The resulting copolymer dispersion contained 20% by weight of a copolymer solid.

#### Preparative Example 8

25 A compound (18 g) represented by  $CF_3CF_2(CF_2CF_2)_nCH_2CH_2OCOC(CH_3)=CH_2$  (a mixture of compounds wherein n is 3, 4 and 5 in a weight ratio of 5:3:1),

10 g of  $CH_2=C(CH_3)COO(CH_2CH_2O)_9CH_3$ ,

7 g of  $CH_2=C(CH_3)COO(CH_2CH(CH_3)O)_9H$ ,

4 g of  $CH_2=C(CH_3)COOCH_2CH(OH)CH_2Cl$ ,

30 1 g of  $CH_2=C(CH_3)COOCH_2CH(OH)CH_2OH$ , 70 g of deoxygenated high purity water, 80 g of isopropanol and 0.04 g of n-laurylmercaptane were charged in a four-necked glass flask equipped with a mercury thermometer and a stirrer of a tetrafluoroethylene crescent-shaped stirrer, and then sufficiently dispersed by stirring under a nitrogen flow. After nitrogen was blown through the flask for about 1 hour, a solution prepared by dissolving 0.4 g of azobisisobutyramidine hydrochloride in 10 g of water was added and the copolymerization reaction was conducted under a nitrogen flow at 60°C. for 10 hours. A gas chromatography analysis revealed that a conversion rate of the copolymerization reaction is not smaller than 99%. This conversion rate showed that the proportion of repeating units in the resulting copolymer is almost the same as that of the charged monomers. The resulting copolymer dispersion contained 20% by weight of a copolymer solid.

#### Preparative Example 9

55  $CF_3(CF_2)_7CH_2CH_2OCOCH=CH_2$  (60% by weight) (90 g), methacrylonitrile (12% by weight) (18 g),  $CH_2=C(CH_3)COO(CH_2CH_2O)_9H$  (15% by weight) (22.5 g),  $CH_2=C(CH_3)COO(CH_2CH_2O)_{4.5}H$  (10% by weight) (15 g), hydroxyethyl methacrylate (3% by weight) (4.5 g), 450 g of deoxygenated deionized water, 100 g of acetone, 1.5 g of azobisisobutyramidine dihydrochloride and 10 g of



60 were charged in a four-necked glass flask equipped with a mercury thermometer and a stirrer of a tetrafluoroethylene

crescent-shaped stirrer, and then sufficiently emulsified by stirring under a nitrogen flow. After nitrogen was blown through the flask for about 1 hour, the copolymerization reaction was conducted with slowly stirring at 60° C. for 20 hours. A gas chromatography analysis revealed that a conversion rate of the copolymerization reaction is not smaller than 99.6% (based on the fluoroalkyl group-containing polymerizable compound). The resulting stable emulsified latex contained 22.5% by weight of a copolymer solid.

#### Preparative Example 10

A monomer/emulsifier/water mixture of a compound (32.0 g) represented by  $\text{CF}_3\text{CF}_2(\text{CF}_2\text{CF}_2)_n\text{CH}_2\text{CH}_2\text{OOCCH}=\text{CH}_2$  (a mixture of compounds wherein n is 3, 4 and 5 in a weight ratio of 5:3:1), 80 g of  $\text{CH}_2=\text{C}(\text{CH}_3)\text{COO}[\text{CH}_2\text{CH}(\text{CH}_3)\text{O}]_7-(\text{CH}_2\text{CH}_2\text{O})_9-$   $\text{C}_8\text{H}_{17}$ , 1.5 g of polyoxyethylene oleyl ether, 0.25 g of trimethylstearyl ammonium chloride, 10.0 g of ethyl acetate and 121.3 g of deionized water was emulsified by a high-pressure homogenizer. Then, 50 g of the resulting emulsion, 0.24 g of azobisisobutyronitrile and 0.12 g of tert-dodecylmercaptane were charged in a 100 ml glass ampul. After replacing the vapor phase by nitrogen, the copolymerization was conducted at 60° C. for 12 hours. The resulting emulsion was diluted with deionized water to adjust the solid content to 20.0%.

#### EXAMPLE 1

The copolymer dispersion prepared in Preparative Example 6 was diluted with water so that the copolymer solid content was 0.5% by weight. The acetylated cotton obtained in Preparative Example 1 was immersed in the diluted liquid and squeezed with a roll to adjust a wet pickup to 70%. Then, the acetylated cotton was dried at 100° C. for 3 minutes and treated at 160° C. for 1 minute.

With respect to the cloth thus treated, the water repellency was 7, the oil repellency was 7, and the soil release property was 5.

#### EXAMPLES 2 to 17

Except that the cloths treated in the first step of Examples 1 to 5 were treated with the copolymer dispersions prepared in Preparative Examples 6 to 10, the same manner as in Example 1 was repeated. The evaluation results are shown in Table 4.

#### Comparative Examples 1 to 5

Except that the cotton cloths which were not subjected to the treatment of the first step were treated with the copolymer dispersions prepared in Preparative Examples 6 to 10, the same manner as in Example 1 was repeated. The evaluation results are shown in Table 4.

TABLE 4

|           | First step  | Second step, copolymer | Water repellency No. | Oil repellency No. | Soil release property |
|-----------|-------------|------------------------|----------------------|--------------------|-----------------------|
| Example 1 | Preparative | Preparative            | 70                   | 7                  | 5                     |
|           | Example 1   | Example 6              |                      |                    |                       |
| Example 2 | Preparative | Preparative            | 70                   | 7                  | 5                     |
|           | Example 1   | Example 7              |                      |                    |                       |
| Example 3 | Preparative | Preparative            | 50                   | 6                  | 5                     |
|           | Example 1   | Example 8              |                      |                    |                       |

TABLE 4-continued

|             | First step  | Second step, copolymer | Water repellency No. | Oil repellency No. | Soil release property |
|-------------|-------------|------------------------|----------------------|--------------------|-----------------------|
| Example 4   | Preparative | Preparative            | 50                   | 6                  | 5                     |
| Example 5   | Preparative | Example 9              | 70                   | 6                  | 4                     |
|             | Example 1   | Preparative            | Example 10           |                    |                       |
| Example 6   | Preparative | Preparative            | 70                   | 6                  | 5                     |
|             | Example 2   | Example 6              |                      |                    |                       |
| Example 7   | Preparative | Preparative            | 50                   | 6                  | 5                     |
|             | Example 2   | Example 7              |                      |                    |                       |
| Example 8   | Preparative | Preparative            | 50                   | 6                  | 5                     |
|             | Example 2   | Example 8              |                      |                    |                       |
| Example 9   | Preparative | Preparative            | 70                   | 6                  | 5                     |
|             | Example 3   | Example 6              |                      |                    |                       |
| Example 10  | Preparative | Preparative            | 50                   | 6                  | 5                     |
|             | Example 3   | Example 7              |                      |                    |                       |
| Example 11  | Preparative | Preparative            | 50                   | 5                  | 5                     |
|             | Example 3   | Example 8              |                      |                    |                       |
| Example 12  | Preparative | Preparative            | 70                   | 6                  | 5                     |
|             | Example 4   | Example 6              |                      |                    |                       |
| Example 13  | Preparative | Preparative            | 70                   | 6                  | 5                     |
|             | Example 4   | Example 7              |                      |                    |                       |
| Example 14  | Preparative | Preparative            | 50                   | 5                  | 5                     |
|             | Example 4   | Example 8              |                      |                    |                       |
| Example 15  | Preparative | Preparative            | 70                   | 6                  | 5                     |
|             | Example 5   | Example 6              |                      |                    |                       |
| Example 16  | Preparative | Preparative            | 70                   | 6                  | 5                     |
|             | Example 5   | Example 7              |                      |                    |                       |
| Example 17  | Preparative | Preparative            | 70                   | 6                  | 5                     |
|             | Example 5   | Example 8              |                      |                    |                       |
| Comparative | —           | Preparative            | 50                   | 4                  | 2                     |
| Example 1   | —           | Example 6              |                      |                    |                       |
| Comparative | —           | Preparative            | 50                   | 4                  | 2                     |
| Example 2   | —           | Example 7              |                      |                    |                       |
| Comparative | —           | Preparative            | 50                   | 4                  | 2                     |
| Example 3   | —           | Example 8              |                      |                    |                       |
| Comparative | —           | Preparative            | 50                   | 3                  | 1                     |
| Example 4   | —           | Example 9              |                      |                    |                       |
| Comparative | —           | Preparative            | 50                   | 4                  | 1                     |
| Example 5   | —           | Example 10             |                      |                    |                       |

We claim:

1. A method of stainproofing a cellulose fiber, which comprises the steps of:
  - (1) esterifying a portion of the hydroxyl groups of the cellulose fiber in a heterogeneous reaction system such that the degree of esterification as represented by a degree of substitution is from 0.01 to 1.5; and then
  - (2) treating the partially esterified cellulose fiber with a solution or emulsion of a copolymer having repeating units derived from a fluoroalkyl group-containing polymerizable compound and a compound represented by the general formula:



wherein X is  $-\text{CH}(\text{CH}_3)-\text{CH}_2-$  or  $-\text{CH}_2\text{CH}(\text{CH}_3)-$ ; Y is  $-\text{CH}_2\text{CH}_2-$ ;  $\text{R}^1$  is a hydrogen atom or a methyl group;  $\text{R}^2$  is a hydrogen atom or an alkyl group having 1 to 8 carbon atoms; and each of m and n is an integer of 0 to 50, provided that the total of m and n is an integer of 1 to 70.

2. A cellulose textile obtained by esterifying a portion of the hydroxyl groups of the cellulose fiber in a heterogeneous reaction system such that the degree of esterification as represented by a degree of substitution is from 0.01 to 1.5 and then subjecting the partially esterified cellulose fiber to a stainproofing treatment with a solution or emulsion of a copolymer having repeating units derived from a fluoroalkyl group-containing polymerizable compound and a compound represented by the general formula:

**11**

(I)

wherein X is  $-\text{CH}(\text{CH}_3)-\text{CH}_2-$  or  $-\text{CH}_2\text{CH}(\text{CH}_3)-$ ; Y is  $-\text{CH}_2\text{CH}_2-$ ;  $\text{R}^1$  is a hydrogen atom or a methyl group;  $\text{R}^2$  is a hydrogen atom or an alkyl group having 1 to 8 carbon atoms; and each of m and n is an integer of 0 to 50, provided that the total of m and n is an integer of 1 to 70.

3. The method according to claim 1, wherein the degree of esterification is from 0.03 to 1.3.

4. The cellulose textile according to claim 2, wherein the degree of esterification is from 0.03 to 1.3.

5. The method according to claim 1, comprising esterifying at room temperature to 120° C.

6. The method according to claim 5, comprising esterifying at room temperature to 80° C.

7. The method according to claim 1, wherein the fluoroalkyl group-containing polymerizable compound is represented by the formula:



wherein Rf is a fluoroalkyl group;  $\text{A}^1$  is  $-(\text{CH}_2)_1-$ ,



R is a hydrogen atom or an alkyl group having 1 to 4 carbon atoms, and 1 is from 1 to 10; and  $\text{A}^2$  is a hydrogen atom or a methyl group.

8. The cellulose textile according to claim 2, wherein wherein the fluoroalkyl group-containing polymerizable compound is represented by the formula:



wherein Rf is a fluoroalkyl group;  $\text{A}^1$  is  $-(\text{CH}_2)_1-$ ,

**12**

-continued



5

R is a hydrogen atom or an alkyl group having 1 to 4 carbon atoms, and 1 is from 1 to 10; and  $\text{A}^2$  is a hydrogen atom or a methyl group.

9. The method according to claim 1, wherein the copolymer contains the fluoroalkyl group-containing polymerizable compound in an amount within a range of from 5 to 95% by weight based on the total weight of the copolymer.

10. The method according to claim 9, wherein the copolymer contains the fluoroalkyl group-containing polymerizable compound in an amount within a range of from 30 to 80% by weight based on the total weight of the copolymer.

11. The method according to claim 10, wherein the copolymer contains the fluoroalkyl group-containing polymerizable compound in an amount within a range of from 40 to 70% by weight based on the total weight of the copolymer.

12. The cellulose textile according to claim 2, wherein the copolymer contains the fluoroalkyl group-containing polymerizable compound in an amount within a range of from 5 to 95% by weight based on the total weight of the copolymer.

13. The cellulose textile according to claim 12, wherein the copolymer contains the fluoroalkyl group-containing polymerizable compound in an amount within a range of from 30 to 80% by weight based on the total weight of the copolymer.

14. The cellulose textile according to claim 13, wherein the copolymer contains the fluoroalkyl group-containing polymerizable compound in an amount within a range of from 40 to 70% by weight based on the total weight of the copolymer.

\* \* \* \* \*